

**[54] ULTRASONIC WAVE DELAY LINE**

[75] Inventors: **Takahiro Inamura; Masao Ohno; Munehisa Tsunekawa; Yasuyuki Nakata**, all of Tokyo, Japan

[73] Assignees: **Nippon Telegraph & Telephone Public Corporation; Nippon Kogaku K.K.**, both of Tokyo, Japan

[22] Filed: **Sept. 2, 1971**

[21] Appl. No.: **177,420**

**Related U.S. Application Data**

[63] Continuation-in-part of Ser. No. 811,964, April 1, 1969, abandoned.

**[30] Foreign Application Priority Data**

Apr. 5, 1968 Japan ..... 43/22126

[52] U.S. Cl. ..... 333/30 R, 106/53

[51] Int. Cl. ..... H03h 7/30, C03c 3/10, C03c 3/04

[58] Field of Search ..... 106/53; 333/30

**[56] References Cited****UNITED STATES PATENTS**

2,367,871 1/1945 Kalsing et al. ..... 106/53

3,154,425 10/1964 Hoover et al. ..... 106/53  
3,173,780 3/1965 Hoover ..... 106/53

**FOREIGN PATENTS OR APPLICATIONS**

1,807,831 8/1969 Germany ..... 106/53  
2,025,441 1/1971 Germany ..... 106/53

*Primary Examiner*—A. B. Curtis

*Assistant Examiner*—Mark Bell

*Attorney*—Anton J. Wille

**[57] ABSTRACT**

An ultrasonic wave delay line comprising a delaying medium made up of a glass having a composition of, by weight, 57 to 78 percent  $\text{SiO}_2$ , 0.5 to 9 percent  $\text{Al}_2\text{O}_3$ , 16 to 19 percent  $\text{PbO}$ , up to 11 percent  $\text{Na}_2\text{O}$ , and up to 20 percent  $\text{K}_2\text{O}$ , the combined amounts of  $\text{Na}_2\text{O} + \text{K}_2\text{O}$  being 9 to 20 percent and having temperature coefficient of time delay of not more than  $5 \times 10^{-6}/^\circ\text{C}$  in a wide temperature range, and an acoustic attenuation factor of less than  $10 \times 10^{-3}$  dB per cycle above 1 MHz.

**6 Claims, 2 Drawing Figures**

FIG. 1



FIG. 2



## ULTRASONIC WAVE DELAY LINE

The present application is a continuation-in-part of U.S. application Ser. No. 811,964 filed Apr. 1, 1969 now abandoned.

## BACKGROUND OF THE INVENTION

## 1. Field of the Invention

The present invention relates to an ultrasonic wave delay line employing as the delaying medium a glass having a novel composition and excellent characteristics.

## 2. Description Of The Prior Art

Generally, an ultrasonic wave delay line comprises a medium for transmitting ultrasonic waves therethrough, a transducer disposed upon a suitable portion of the surface of the medium for transducing electrical signals into mechanical ones and another transducer adapted to convert the mechanical signals to electrical ones. The simplest construction of the delay line of the type described comprises an input transducer and an output transducer attached to the respective ends of a medium. By the input transducer electrical signals are converted into mechanical signals (shear mode ultrasonic waves) which in turn transmit through the medium and reach the output transducer where the mechanical signals are again converted into the electrical signals. In this case, the signals are delayed by the time required for the mechanical signals to pass through the medium. That is, the delay time is defined as the time difference between the input and the output signals.

The characteristics of the delay line are dependent upon the delay time, the temperature coefficient of the delay time, and the amount of attenuation of the signals, etc. Various delay mediums having different shapes and being made of various materials have been proposed.

Generally the delay mediums are made of quartz, glass, ceramics, metals and the like; and mediums of the multireflection type have been also proposed to provide a compact delay line capable of increasing the delay time.

The ultrasonic wave delay lines find many applications in the various fields such as television, radar, band width compression, electronic computers and so on. In this case, the delay lines are required to have a smaller temperature coefficient of the delay time and less attenuation of the signals in the delaying medium. The conventional delay mediums made of molten quartz has a temperature coefficient of time delay of the order of about  $8 \times 10^{-5}/^{\circ}\text{C}$ , which is not sufficient for the use in the PAL system color television which requires a temperature coefficient of less than  $3 \times 10^{-6}/^{\circ}\text{C}$ . The problem has not been so far satisfactorily solved because even the improved glass material exhibits a temperature coefficient of  $(1 \text{ to } 5) \times 10^{-5}/^{\circ}\text{C}$ . In the case of a multi-reflection type delay mediums, a precise machining operation is required so that glass is advantageous because of its machinability.

As to attenuation, quartz has the least attenuation factor among the glasses with a value of  $2 \times 10^{-4}$  dB per cycle in measurements above 1 MHz. In case of ordinary glass, the attenuation factor is of the order of  $10 \times 10^{-3}$  to  $50 \times 10^{-3}$  dB, which is far from the value satisfactorily applied in practice.

## SUMMARY OF THE INVENTION

In view of the above the primary object of the present invention is to provide an ultrasonic wave delay line having a smaller temperature coefficient of time delay and a smaller signal attenuation factor than heretofore attainable.

According to the present invention, the temperature  $T_o$  at which the delay time becomes minimum can be varied even in the temperature range slightly deviated from the normal temperature by suitably selecting the composition of the ultrasonic wave transmission medium. For example, when the service temperature range is from  $-60$  to  $+90$   $^{\circ}\text{C}$ , the temperature coefficient of delay time of the delay line of the present invention can be made less than  $1.5 \times 10^{-6}/^{\circ}\text{C}$ .

In brief, the present invention provides an ultrasonic wave delay line incorporating a delaying medium made of a glass having the composition of, by weight, 57 to 78 percent  $\text{SiO}_2$ ; 0.5 to 9 percent  $\text{Al}_2\text{O}_3$ ; 16 to 19 percent  $\text{PbO}$ ; up to 11 percent  $\text{Na}_2\text{O}$  and upto 20 percent  $\text{K}_2\text{O}$ ; the combined amounts of  $\text{Na}_2\text{O}$  and  $\text{K}_2\text{O}$  being from 9 to 20 percent, and having a temperature coefficient of time delay of not more than  $5 \times 10^{-6}/^{\circ}\text{C}$  over a wide temperature range centered around room temperature, and an acoustic attenuation factor of less than  $10 \times 10^{-3}$  dB per cycle about 1 MHz. In the foregoing embodiment, a desired temperature coefficient of time delay is  $1 \times 10^{-6}/^{\circ}\text{C}$  to  $5 \times 10^{-6}/^{\circ}\text{C}$ . In the foregoing embodiment a suitable amount of  $\text{K}_2\text{O}$  is 1 to 7 weight percent. In the foregoing embodiment a suitable amount of  $\text{Na}_2\text{O}$  is 6 to 11 weight percent. In the foregoing embodiment a desired amount of  $\text{SiO}_2$  is 60 to 67 weight percent. Also, in the foregoing embodiment the desired amount of  $\text{PbO}$  is 17 weight percent.

The temperature coefficient of time delay can be controlled by the composition of the glass when it is cooled sufficiently gradually, but generally varies depending upon the temperature range selected. The relation between the time delay  $\tau$  and the deviation  $\Delta\tau$  due to temperature difference can be expressed by

$$\Delta\tau/\tau = \alpha (T - T_o)^2$$

where  $\alpha$  = a constant;

45  $T_o$  = temperature at which the delay time is minimum;  
and  $T$  = temperature measured.

It is seen from the equation that in order to reduce the temperature coefficient, it is required that  $T_o$  must be at the middle of the selected service temperature.

55 In the glass of the present invention having the composition described above, the ingredients  $\text{SiO}_2$ ,  $\text{Al}_2\text{O}_3$  and  $\text{PbO}$  have the characteristic of shifting  $T_o$  to the positive side;  $\text{Al}_2\text{O}_3$  has a great influence in this respect while  $\text{PbO}$  has a small influence. On the other hand,  $\text{Na}_2\text{O}$  and  $\text{K}_2\text{O}$  have the tendency of shifting  $T_o$  to the negative side. Of the two,  $\text{Na}_2\text{O}$  is stronger than  $\text{K}_2\text{O}$ . Therefore, by suitably selecting the ratios of these ingredients, the temperature  $T_o$  may be centered in the service temperature range.

60 However, the delay line is used generally at room temperature so that when  $(\text{Na}_2\text{O} + \text{K}_2\text{O})$  is in excess of 20 percent by weight, the amount of the remaining ingredients is not sufficient enough to shift the temperature  $T_o$  to the positive side, thereby lowering the temperature  $T_o$  to a temperature far lower than room temperature. On the other hand, when  $(\text{Na}_2\text{O} + \text{K}_2\text{O})$  is

less than 9 percent by weight, the temperature  $T_o$  will be increased far higher than room temperature. Thus, when  $(Na_2O + K_2O)$  is between 9 percent and 20 percent by weight, a suitable combination of other ingredients of 57 to 78 percent by weight of  $SiO_2$ ; 16 to 19 percent by weight of  $PbO$ ; and 0.5 to 9 percent by weight of  $Al_2O_3$  can set the temperature  $T_o$  close to room temperature.

According to the present invention, in addition to the above described ingredients, less than 10 percent by weight of glass forming oxides or fluorides such as  $Sb_2O_3$  or  $As_2O_3$  may be added as a clarifier.

#### BRIEF DESCRIPTION OF THE DRAWINGS

The present invention will be described in more detail with reference to the accompanying drawings in which:

FIG. 1 shows a typical bar-shaped delay line; and

FIG. 2 is a graph illustrating the relation between the rate of change of delay time and temperature of examples of this invention.

#### DESCRIPTION OF THE PREFERRED EMBODIMENTS

In Table 1 are shown the compositions (No. 1 to No. 25 9) of the glasses embodying the present invention with the ingredients being within the above described ranges and compositions (No. 10 to No. 12) of ordinary glass (flint glass); and the corresponding temperature coefficients of time delay over the temperature range of 0° to 50° C.

TABLE 1.—COMPOSITIONS IN PERCENT BY WEIGHT

| Glass No.                                             | 1     | 2     | 3    | 4     | 5     | 6    | 7    | 8    | 9     | 10    | 11    | 12    |
|-------------------------------------------------------|-------|-------|------|-------|-------|------|------|------|-------|-------|-------|-------|
| Composition:                                          |       |       |      |       |       |      |      |      |       |       |       |       |
| $SiO_2$                                               | 58.0  | 59.0  | 60.5 | 63.5  | 66.0  | 66.0 | 66.5 | 68.0 | 69.5  | 56.0  | 48.0  | 41.0  |
| $Al_2O_3$                                             | 4.5   | 3.5   | 8.5  | 5.0   | 2.5   | 2.5  | 2.5  | 0.5  | 2.5   | ----- | ----- | ----- |
| $Na_2O$                                               | 4.0   | ----- | 10.5 | 6.0   | 6.0   | 3.0  | 6.0  | 6.0  | 9.0   | 4.0   | 4.0   | ----- |
| $K_2O$                                                | 12.5  | 19.5  | 1.5  | 6.5   | 6.5   | 9.0  | 6.0  | 6.5  | ----- | 7.0   | 6.0   | 8.0   |
| $PbO$                                                 | 19.0  | 16.0  | 17.0 | 17.0  | 17.0  | 17.0 | 17.0 | 17.0 | 17.0  | 32.5  | 41.5  | 50.5  |
| $Sb_2O_3$                                             | 1.0   | 1.0   | 1.0  | 0.9   | 1.0   | 1.0  | 0.9  | 0.9  | 1.0   | ----- | ----- | ----- |
| $As_2O_3$                                             | 1.0   | 1.0   | 1.0  | 0.5   | 1.0   | 1.0  | 0.5  | 0.5  | 1.0   | 0.5   | 0.5   | 0.5   |
| F                                                     | ----- | ----- | 0.6  | ----- | ----- | 0.6  | 0.6  | 0.6  | ----- | 25    | 34    | 24    |
| Temperature coefficient in $\times 10^{-6}/^{\circ}C$ | 2     | 3     | 1    | 1     | 1     | 3    | 1    | 2    | 5     | ----- | ----- | ----- |

As will be clearly seen from Table 1, all glasses of the present invention have smaller temperature coefficients of delay time than that of the ordinary glasses, the attenuation factors have been measured to be less than  $10 \times 10^{-3}$  dB per cycle above 1 MHz. For example, glass No. 5 has an attenuation factor of  $8 \times 10^{-3}$  dB per cycle when measured at a frequency of 5 MHz.

The relations between the temperature and the rate of change in delay time of the glass of Table 1 are shown in FIG. 2, and the temperature coefficients of delay times obtained from these curves are shown in Table 2.

TABLE 2

| Glass Nos. | Temperature coefficients in $\times 10^{-6}/^{\circ}C$ . |              |              | $\alpha ( \times 10^{-3}/^{\circ}C.)$ | $T_o (^{\circ}C.)$ |
|------------|----------------------------------------------------------|--------------|--------------|---------------------------------------|--------------------|
|            | 0 to 50° C.                                              | 15 to 65° C. | 30 to 80° C. |                                       |                    |
| 5-----     | 1.0                                                      | 1.8          | 2.5          | 2.3                                   | 4.5                |
| 7-----     | 1.3                                                      | 2.1          | 4.6          | 8.8                                   | 28.0               |
| 4-----     | 1.0                                                      | 0.6          | 1.3          | 3.6                                   | 37.5               |
| 6-----     | 2.7                                                      | 1.6          | 0.7          | 4.0                                   | 59.5               |

There is a relation of  $\Delta\tau/\tau = \Delta (T - T_o)$  as described before so that it is preferable to use the glass having a specific temperature  $T_o$  in such a temperature range from  $T_1$  °C to  $T_2$  °C which satisfies approximately the relation of  $2T_o = T_1 + T_2$  as is clearly seen from FIG. 2 and Table 2. For example, in case of the glass, Nos. 5 and 7 in Table 2, the service temperature range is from 0 to 50° C; in case of No. 4, from 15° to 65° C; and in case of No. 6, from 30° to 80° C.

The present invention has been so far described with particular reference to some embodiments thereof, but it will be understood that variations and modifications can be effected without departing from the true spirit of the present invention.

We claim:

1. An ultrasonic delay line comprising a glass delay medium having a temperature coefficient of time delay of not more than  $5 \times 10^{-6}/^{\circ}C$  and an attenuation factor of less than  $10 \times 10^{-3}$  dB per cycle above 1 MHz, and input and output transducers sealed to the facets on the delay medium, said delay medium consisting essentially of, by weight, 57 - 78 percent  $SiO_2$ , 0.5 to 9 percent  $Al_2O_3$ , 16 to 19 percent  $PbO$ , up to 11 percent  $Na_2O$ , and up to 20 percent  $K_2O$ , the combined amounts of

$Na_2O$  and  $K_2O$  being 9 to 20 percent.

2. An ultrasonic delay line according to claim 1, wherein the temperature coefficient of time delay of  $1 \times 10^{-6}/^{\circ}C$  to  $5 \times 10^{-6}/^{\circ}C$ .

3. An ultrasonic delay line according to claim 1, wherein the amount of  $K_2O$  is 1 to 7 weight percent.

4. An ultrasonic delay line according to claim 1, wherein the amount of  $Na_2O$  is 6 to 11 weight percent.

5. An ultrasonic delay line according to claim 1, wherein the amount of  $SiO_2$  is 60 to 67 weight percent.

6. An ultrasonic delay line according to claim 1, wherein the amount of  $PbO$  is 17 weight percent.

\* \* \* \* \*